

Sept. 28, 1948.

G. R. BURKHARDT  
NOBLE GAS METALLURGY

2,450,081

Filed April 5, 1945

2 Sheets-Sheet 1



FIG.1.



FIG.2.

INVENTOR  
GEORGE R. BURKHARDT  
BY

*George R. Burkhardt* ATTY

Sept. 28, 1948.

G. R. BURKHARDT  
NOBLE GAS METALLURGY

2,450,081

Filed April 5, 1945

2 Sheets-Sheet 2



FIG. 3.

INVENTOR  
GEORGE R. BURKHARDT

BY

*George R. Burkhardt*  
AT&T

## UNITED STATES PATENT OFFICE

2,450,081

NOBLE GAS METALLURGY

George R. Burkhardt, Chicago, Ill.

Application April 5, 1945, Serial No. 586,809

4 Claims. (Cl. 148—16.7)

1

This application is a continuation in part of my pending application, Serial No. 523,705, filed February 24, 1944, Patent No. 2,426,814, for "Noble gas metallurgy."

The present invention relates to a method for the treatment of a ferrous metal or iron-carbon alloy and more particularly to an improvement in the metallurgy of steel by which a more compact and more minute crystalline structure is obtained. By means of the improved method as hereinafter described, dissolved embrittling gases, slag inclusions and other stress raisers are removed from the metal to an extent which is not possible by other methods heretofore used.

The usual practice in the manufacture of iron-carbon alloys, or steel, results in a metal structure in which small amounts of slag are included, and in which dissolved gases, such as hydrogen, oxygen and other chemically active gases, are present which substantially reduce the strength of the metal.

In the manufacture of steel by the Bessemer process and the open-hearth process, it is difficult to control the grain size of the product for the reason that the grain size is dependent to a considerable extent on the amount of slag inclusions and other impurities present. When metal produced by either of these processes is poured into molds or ingots, the metal contracts during cooling and solidification, by which cavities, known as "pipes" are formed, which frequently extend into the ingot such a distance that they are not removed when the top of the ingot or casting is cut off preparatory to the rolling operations.

In these processes, spiegeleisen or ferromanganese is added for the purpose of supplying the proper percentages of manganese and carbon in the steel so as to obtain the desired rolling properties. It is known, however, that while the manganese of the spiegeleisen or ferromanganese combines with dissolved oxygen in the metal and serves to decrease the blow-holes in the solid ingot, such blow-holes are invariably present and substantially weaken the metal. The presence of small proportions of slag also decreases the strength of the metal by preventing the complete union of metal particles in the steel. It is known also that the presence of small proportions of slag in the metal affects the crystallization or grain size of crystals in the metal.

Attempts have been made to remove oxidizing gases in ferrous metals as by introducing a blast of a noble gas into the converter to displace air from the metal prior to the introduction of hy-

2

drogen, which is employed for the purpose of reducing the oxides present in the metal. Such use of a noble gas as a scavenger to remove oxygen prior to the introduction of hydrogen has no substantial effect, however, on the physical or chemical properties of the metal. Attempts have also been made to employ nitrogen, helium, and other rare gases, by bubbling the gas through the molten metal to produce agitation, but no substantial improvement in the physical properties of the metal has been obtained by this bubbling method, and neither of these prior methods has met with commercial acceptance.

It has been found that steel rails rolled from blooms or ingots which have been re-heated by the usual prior art methods frequently develop fissures because the metal has been made minutely porous by effused gases.

The present invention in the treatment of ferrous metal or iron-carbon alloys involves the use of a blanket or atmosphere of a noble gas which is preferably employed at a high pressure and which surrounds the ingot or metal under treatment for a substantial period of time during which the metal is allowed to remain quiescent, so as to permit occluded or dissolved gases in the metal to be dispersed into the noble gas, whereby they may be substantially completely removed from the metal. The dissolved gases generally include oxygen, nitrogen and carbon monoxide, which become dispersed or diffused into the body of the noble gas. The use of a noble gas as a blanket or atmosphere around the metal, permits the use of substantially elevated temperatures to be maintained without oxidizing effect on the metal and allows the dissolved and occluded gases therein to be gradually removed from the metal, resulting in the substantial elimination of blow-holes in the metal without deleterious action on the metal under treatment. As herein-after explained, the noble gas, as helium, may be independently heated and the maintenance of the temperature during treatment and the subsequent cooling of the metal in the noble gas atmosphere may be independently regulated, whereby the grain size of the crystals in the final metal product may be more completely controlled.

It will be understood that the method of the present invention relates particularly to the treatment of the hot solid metal containing austenite, in the form of a casting or ingot, and may be employed directly in the treatment of molten metal from a Bessemer converter or open-hearth in a ladle or prior to the casting of the ingot, or 55 it may be applied directly to cast ingots which

have cooled and which may be reheated to the desired temperature for treatment at which austenite is present. In the treatment of the molten metal, the amount of slag present may amount to as much as 2%, for example, which while the metal is molten gradually rises to the surface and may be drawn off prior to the solidification of the metal, thus greatly improving the welding properties and tensile strength thereof.

The invention preferably involves the use of a blanket or atmosphere of helium, although any other noble gas, or member of the helium family, as argon, neon, zenon or krypton, may be used, or a mixture of two or more of these gases may be employed. The noble gas may be independently heated during the treatment of the metal, or prior thereto, or the metal under treatment may be separately heated to provide a temperature of the steel or iron-carbon alloy at which austenite is present, so as to maintain the metal at a desired temperature during a period of quiescence in which dissolved or occluded gases in the metal may be dispersed into or taken up by the noble gas. It has been found preferable to subject the ferrous metal during a period of quiescence to an atmosphere of the noble gas both before and after it is rolled, and permitting the metal to cool in an atmosphere of the noble gas, as the metal adsorbs injurious gases if subjected to atmospheric air during slow cooling.

The importance of reheating or soaking an ingot or casting in a noble gas is apparent from a comparison of the physical properties and microstructure of steels treated by this method with those of steels treated by the ordinary methods heretofore used. The improvement in the properties is believed to be associated with a change in space lattice or porosity of the metal which takes place when the metal is heated to the temperature at which austenite is formed. This change in space lattice or porosity of the metal generally takes place between 1330° F. and 2550° F., between which temperatures austenite occurs in simple steels having less than about 1.7% of carbon. It will be understood, of course, that austenite is a solid solution of carbon in gamma iron, and occurs between the "solidus" and the "liquidus" of the equilibrium diagram for iron-carbon alloys.

In the method of the invention, helium gas is preferably employed under a pressure of from about 1000 to 4000 pounds pressure per square inch, the temperature of the gas being controlled by the addition of heat, if necessary, so as to maintain the metal during the period of quiescence in the condition in which austenite is present, during which the pores of the metal are open and the occluded and dissolved gases in the metal may be readily removed therefrom by being dispersed or dissipated into the body of the helium or other noble gas employed.

The heat conductivity of helium is greater than that of any other gas with the exception of hydrogen, which follows from the kinetic theory of gases, since except for hydrogen it has the smallest molecular weight of any gas and therefore the highest molecular velocities at a given temperature. Helium transfers its kinetic energy, therefore, from molecule to molecule more rapidly than any other gas, with the exception of hydrogen. The thermal conductivity of helium is .000339 at 0° C., as compared with .0000568 for air at 0° C. The thermal conductivity of helium is therefore about six times that of air, so that heat may be added to or abstracted

from a metal by means of helium about six times as rapidly as with air, and the helium has the advantage, furthermore, that the metal is unaffected thereby at any temperature, whereas in the presence of air, the metal is oxidized to a substantial extent at high temperatures.

The heat conductivity of a gas is independent of pressure through a wide range, and in cooling the metal in contact with helium, or other noble gas, in accordance with this invention, the gas operates as a protecting layer and prevents access of chemically active gases, such as air, until the metal is cold, or cooled to the extent that it is unaffected by the air at room temperature. It will be understood that helium and other gases of the helium family are monatomic, that is, the molecules of these gases are atoms and do not dissociate to form atoms in the nascent state so as to react chemically with other materials. Hydrogen, on the other hand, is diatomic, that is, the molecule of hydrogen, H<sub>2</sub>, is composed of two atoms of hydrogen, H<sup>-</sup>, having a single bond or valence, so that when the gas dissociates to form the hydrogen atoms, it readily reacts chemically with other substances present. The noble gases, unlike most other gases, are inert and are not dissolved or occluded in metals and do not enter into chemical combination with the metals or other materials present under the conditions of operation in the treatment of metals in accordance with the invention hereinafter more fully described.

In carrying out the method of the invention, the noble gas, as helium, may be purified and recycled during the operation or treatment, or purified periodically from time to time as required, depending upon the particular metal composition treated, or the amount of dissolved and absorbed gases in the metal treated. The method of purification to be employed depends, to some extent, on the particular conditions of operation, but ordinarily the gas may be purified by first passing it through soda-lime, in order to remove carbon dioxide, then through calcium chloride to remove water vapor, then through heated copper to remove oxygen, and also to remove hydrogen, if present, by combination with oxygen to form water vapor, then through calcium chloride to remove water vapor, if present, and finally over heated magnesium or calcium to remove nitrogen.

It will be understood that a gas, exclusive of the noble gases, when in contact with a metal is held in contact with the surface thereof through molecular forces which produce more or less condensation of the gas on the surface of the metal. The gas also permeates the pores of the metal and is condensed on the surfaces of the pores, which phenomenon is referred to as "occlusion." When steel is subjected to an atmosphere of a noble gas, as helium, at a temperature at which austenite is present in the steel, the gases held on the surface of the metal and in the pores by condensation and occlusion are gradually diffused into the body or blanket of the noble gas, following the law of diffusion of gases into each other, so that the condensed and occluded gases are progressively removed by the noble gas. If the noble gas is heated to a higher temperature than that of the metal under treatment, the heat from the gas is rapidly transferred to the ingot or metal because of the high conductivity of the gas, as helium, irrespective of the pressures which are used, and by the removal of the injurious gases, the metal product which is produced is

more compacted and more homogenous than the metal product produced by other prior art methods, since blow-holes are substantially eliminated and the product is not subject to atmospheric corrosion as is the case with steel or iron-carbon alloys produced by methods of the prior art.

One of the objects of the invention is to provide a method for the treatment of iron-carbon alloys in the solid state in which a substantially larger proportion of dissolved or occluded gases may be removed from the metal than by any of the methods heretofore used. In accordance with this object of the invention, the method herein-after described provides for the treatment of the metal in the solid state at a temperature at which austenite is present with a noble gas, as helium, in a manner so that the metal may lie undisturbed or quiescent in the gas for a period of time sufficient to permit occluded and dissolved gases in the metal to be dispersed or dissipated into the body of the surrounding noble gas.

Another object is to provide a method for the treatment of steel or iron-carbon alloys, which permits the casting of ingots or castings by the usual commercial processes, after which the ingots or castings may be subjected in a heated condition to an atmosphere of helium or other noble gas at a temperature at which austenite is present in the metal, the ingot or casting being treated or allowed to remain quiescent in the noble gas for a period of time sufficient to permit dissolved or occluded gases in the metal to be taken up by the body of the noble gas, thereby removing blow-holes from the metal and substantially increasing the tensile strength and other desired properties of the metal.

A further object is to provide a method for the treatment of steel castings or ingots at a temperature at which austenite is present in the metal, by subjecting it to an atmosphere of a noble gas in which the metal may remain in contact with said gas for a period of time sufficient to permit occluded and dissolved gases to be effused from the metal and dispersed into the noble gas, which may thereafter be chemically purified to remove carbon dioxide, water vapor, oxygen, hydrogen, nitrogen and other undesired constituents.

Another object is to provide a method for the treatment of iron-carbon alloys or steel in the solid state, in the form of castings, ingots or blooms, to remove occluded, condensed and dissolved foreign gases, and to eliminate blow-holes and other imperfections in the metal while it remains quiescent in the austenitic condition in a manner such that the metal is compressed or compacted under a high pressure, so that the metal is rendered less subject to corrosion by contact with the atmosphere after it has been cooled.

Another object is to provide a continuous method for the treatment of ingots or steel castings, in which the ingots or castings may be successively treated in hotter and hotter helium, or noble gas, by the abstraction of heat from the ingots or castings as it is passed progressively through the system, and in which the noble gas may be used as a cooling medium for the out-going ingots, by which the ingots may be cooled to room temperature at the out-going end of the system, and whereby heat is abstracted from the ingots or castings by the application of the counter current principle in the system, so that as the treatment of one ingot or casting is completed and is removed from the system at the out-going end, another ingot may be inserted into the system.

at the incoming end of the line, thereby rendering the method substantially continuous.

A still further object is to provide a continuous method for the treatment of steel ingots and castings in a sufficiently heated condition to contain austenite, by subjecting the ingots or castings, as they advance in the system, to successively purer and purer helium, or other noble gas, in a manner to progressively remove occluded, condensed and dissolved foreign gases from the metal, and controlling the cooling of the metal in the noble gas so as not to expose the metal to the atmosphere until it is at a temperature at which the metal is unaffected thereby, whereby the metal is substantially compacted so as to remove blow-holes in the metal and a uniform, fine-grained metal product is obtained.

The invention is explained in detail in connection with various forms of apparatus which may be employed in carrying out the invention, as illustrated in the accompanying drawings, in which:

Figure 1 is an elevational view, partly in section, of an ingot mold illustrating an application of the invention, in which a storage tank for the noble gas and connections to the mold, together with apparatus for purifying the gas, are diagrammatically indicated.

Figure 2 is a plan view of apparatus illustrating the use of the invention in connection with ingots on the conventional ingot car; and

Figure 3 is a view in elevation, partly in section, illustrating the application of the invention to an ingot mold of the bottom poured type.

Referring to the several drawings illustrating various applications of the invention, the procedure in carrying out the novel method in connection with the apparatus shown in Fig. 1 of the drawings is as follows:

As here shown the ingot mold is designated by the reference letter I and to carry out the present invention there is associated with this mold a gas-feeding head 16 designed to be properly fitted over and into the upper end of the mold and provided with a noble gas intake 17, a suitable operated intake valve 18, a combined feeding and exhaust neck 19 snugly fitting within the upper open end of the ingot mold, an exhaust outlet 20 opposite the gas intake 17 and a suitably designed and suitably controlled valve 21 for opening and closing the gas exhaust 20. In explanation of the invention as carried out in connection with an ingot mold and a gas feeding head 16, as is shown in Fig. 1 of the drawings, it is to be noted that the noble gas is contained in suitable supply tanks or tank cars 23, under a high pressure, as from 1000 to 4000 pounds per square inch, and the maintained pressure therein is sufficient to pump out the atmosphere in the mold, or, if desired, supplemental pumping means 36 may be used. In practice the molten metal is poured into the ingot mold I and the gas feeding head 16 is then inserted into the open top of the mold. The valves 18 and 21 are then opened and the air in the mold is displaced by the incoming noble gas, from the pipe 32, after which the valve 21 of the exhaust outlet 20 is closed and the pressure of the noble gas is built up until the metal, cooled to a pasty consistency, is thoroughly compressed by pressure on the top and sides of the ingot. Then, after a predetermined period of soaking the ingot in the heated noble gas, such as a period of from one to five hours, the exhaust valve 21 is opened to permit the noble gas to be collected for reuse.

The gas issuing from the outlet 20 may be con-

ducted through a pipe 34, having a pump 36 therein, and from thence to a purifying apparatus containing chemicals for the removal of impurities from the gas, such as carbon dioxide, water vapor, oxygen, nitrogen, or other gaseous impurities, as hydrogen, which may have been taken up by the helium or other noble gas used while it is in contact with the heated ingot or casting. The carbon dioxide may be removed by the use of soda-lime, for example, in a container 38; water-vapor may be removed from the noble gas by means of calcium chloride in a container 40; oxygen may be removed by means of heated copper in a container 42, in which hydrogen, if present in the gas, will react with the oxygen to form water-vapor, which may then be removed by the use of calcium chloride in an additional container, not shown, and finally, nitrogen present in the gas may be removed by means of magnesium or calcium in a container 44, in a manner well known by those skilled in the art. From the container 44, the gas may be conducted through a pipe 46 to a storage tank 48, from which the gas may be subsequently drawn for treatment of the next ingot in a series, or for treatment of a series of ingots or castings in a system, as hereinafter more fully explained. It is to be understood that the purification steps above described may be varied as may be found desirable, or additional purification steps and other chemicals may be added, and the purification steps above indicated are merely for purposes of illustration. It may be found desirable, to remove oxygen while the gas is in a highly heated condition, and then to remove nitrogen while the gas is still at a high temperature, after which the gas may be cooled somewhat to remove carbon dioxide and water-vapor.

In the illustration of Figure 2, it is to be noted that the ingots on the ingot car 22 are followed by a gas tank 23 mounted on a car 50. It will be understood that during transportation of the ingots in the ingot car 22, helium or other noble gas may be passed through pipe 17 from the tank 23 on the car 50 to the gas feeding head 16, through the intake valve 18, through the feeding and exhaust neck 19 from thence through a bleed valve 52, which may be provided in a casing of the ingot mold I, positioned above the level of the top of the ingot therein, through which air may be expelled during the admission of the helium or noble gas to the mold until helium gas passes out of the opening 52. The point at which the bleed valve at 52 should be closed may be readily determined by spectrometry or by the simple expedient of a lighted match or its equivalent held at the opening 52, since helium or other noble gas will not support combustion. As soon as the lighted match is extinguished, indicating a high proportion of helium issuing from the outlet, the valve at 52 should be closed in order to prevent substantial loss of the noble gas. In the use of a series of ingots on the ingot cars in carrying out the method of the invention, the first mold 16 is first filled with helium, or the noble gas used, and the valve 21 may then be opened whereby the gas then passes through the exit pipe 20 to the ingot mold 16' next in the series, by opening the admission valve 18' and admitting the gas to the ingot chamber. After the ingot mold is filled with the noble gas, the bleed valve, similar to that used at 52, is closed and the gas is then similarly passed to the remaining ingot molds, if any, in the series and the last exhaust valve similar to the valve 21 is

then closed and the pressure in the system is then built up to the desired pressure, such as 2000 pounds per square inch, for example, or generally within the range of from about 1000 to 4000 pounds per square inch. The ingot molds on the tank cars may advantageously be furnished with separate or independent heating elements, such as tungsten rods or coils which may be electrically heated in the usual manner, or the noble gas passing to the first ingot mold 16 may be heated to the desired temperature, generally within the range from about 1330° F. to 2550° F. below the "liquidus" at which temperature range the ingot remains solid, but contains austenite, and the pressure of the gas is regulated to provide the desired pressure in the system. If the ingot molds which are added at the incoming end of the series are in a cold condition, the temperature of the ingots in the series is gradually increased by heat absorbed from the gas passing through the molds in accordance with the counter current principle, the gas at the incoming end, passing to the first mold, being at a temperature such as to heat the ingot therein to a temperature at which austenite is present, that is, without melting the metal. The first ingot mold is permitted to cool in an atmosphere of the noble gas by closing the valves 18 and 21, and then removing the mold with the ingot therein from the series, after which another ingot mold with an ingot therein may be added at the end of the line so as to pass through the system up to the point at which it contacts with fresh helium, or noble gas, so as to be first in the series, whereby in passing through the system the temperature of the ingot is gradually increased and the ingot, while at a temperature at which austenite is present, remains quiescent for a time sufficient to permit occluded and dissolved foreign gases to be evolved or effused from the metal and taken up by the noble gas. As the noble gas passes through the series, it takes up more and more of the dissolved and adsorbed foreign gases, as oxygen, nitrogen and hydrogen, and during the passage forwardly through the series, its temperature is gradually reduced and the pressure may be allowed to be correspondingly reduced, if desired, so that at the end of the series, the noble gas is in a condition in which it may be readily purified by passing through the chemical purifying system as indicated in Fig. 1 of the drawings. The purified gas may then be passed to a storage tank, as 48, and then may be reused in the same or a similar system.

It will be understood that in a large plant, it will be preferable to treat the ingots immediately after the metal is poured from a ladle into the molds, and the ingot molds may be treated on ingot cars in the manner indicated in Fig. 2 of the drawings in a series in the manner above explained, except that it will be unnecessary to separately heat the noble gas, which may be employed to assist in the cooling of the ingots, and may be passed consecutively from the outgoing ingot to the incoming ingot in the line whereby the gas becomes hotter and hotter in passing through the series, taking up more and more impurities in accordance with the counter current principle, the fresh helium gas, or other noble gas, passing to the most purified ingot in a series, which is that ingot which has passed from the incoming end through the series to the outgoing end and is ready to be discharged. It will be understood that the gas may be purified by separate chemical apparatus after having passed

through the series or it may be used for an extended period of time over and over again through several series of treatments until the impurities or foreign gases have accumulated in the noble gas to such an extent as to require purification. Obviously, while the impure gas is being purified, a separate tank of purified noble gas may be used so as not to interfere with the continuous operation of the plant.

In Fig. 3 of the drawings is shown a bottom-fed type of ingot mold designated generally by the letter A and which type of mold lends itself very effectively to the carrying out of the process of the present invention. The procedure in connection with the bottom-fed mold shown in Fig. 5 of the drawings is that the metal is first poured in the gate 24 at the top and rear of the mold. The sides 25 of the riser 26 are made of refractory material to hold in the heat. The refractory material is encased by a cast iron portion 27 integral with the ingot mold A which rests on the usual pouring plate 28. The metal runs into the ingot mold through the opening 29 until the molten metal is at the proper height in the ingot mold. The top B is connected to the bottom by threading, or it may be made integral therewith by welding. The top contains the inlet valve 30 and exhaust valve 31, and may also be provided with the lifting eye 33. The heated helium, or noble gas, which is under a high pressure, compresses or exerts pressure on the ingot from all sides and assists in removing the dissolved and adsorbed gases and causing collapsing of blow-holes in the metal, thus greatly improving the physical properties of the metal. After the ingot has solidified, the gas is pumped off or drawn off and the mold may then be lifted off the ingot by means of a suitable lifting device which may be attached through the opening at the top of the mold, after which the gate on the ingot may be burned off. This type of ingot mold prevents slag from getting into the molds, and prevents metal from spattering up the sides of the mold and forming cold shuts. This form of apparatus is particularly useful for carrying out the improved method of the invention for the reason that the hot gas prevents the top of the ingot from cooling before the bottom portion is cooled, or solidified.

It will be understood that various changes or modifications may be made in the method above described without departing from the spirit or the scope of the invention as defined in the annexed claims.

I claim:

1. In the manufacture of steel, a method for improving the physical properties thereof which comprises subjecting solid steel at a temperature between about 1330° F. and 2550° F., at which austenite is present, to an atmosphere of a noble gas surrounding said steel, said gas being under pressure between about 1,000 and 4,000 pounds per square inch, said steel being surrounded by said atmosphere under said pressure for a substantial period of quiescence during which occluded and dissolved gases in the steel become dispersed into the said noble gas atmosphere, thereafter cooling said steel to ordinary temperatures in said noble gas atmosphere while under said pressure and finally separating said steel from said noble gas atmosphere.

2. In the manufacture of steel, a method for improving the physical properties thereof which comprises subjecting solid steel at a temperature between about 1330° F. and 2550° F., at which austenite is present, to an atmosphere of a noble gas surrounding said steel, said gas being under pressure between about 1,000 and 4,000 pounds per square inch, said steel being surrounded by said atmosphere under said pressure for a substantial period of quiescence during which occluded and dissolved gases in the steel become dispersed into the said noble gas atmosphere, chemically purifying said noble gas to remove impurities therefrom and recycling said noble gas into the process, thereafter cooling said steel to ordinary temperatures in said noble gas atmosphere while under said pressure and finally separating said steel from said noble gas atmosphere.
3. In the manufacture of steel, a method for improving the physical properties thereof which comprises subjecting solid steel at a temperature between about 1330° F. and 2550° F., at which austenite is present, to an atmosphere of substantially pure helium surrounding said steel, said helium being under pressure between about 1,000 and 4,000 pounds per square inch, said steel being surrounded by said helium at said temperature and under said pressure for a substantial period of quiescence during which occluded and dissolved gases in the steel become dispersed into said helium atmosphere, thereafter cooling said steel to ordinary temperatures in said helium atmosphere while under said pressure and finally separating said steel from said helium atmosphere.
4. In the manufacture of steel, a continuous method for improving the physical properties thereof which comprises subjecting solid steel ingots in a series at a temperature between about 1330° F. and 2550° F., at which austenite is present, to an atmosphere of substantially pure helium under pressure between about 1,000 and 4,000 pounds per square inch, said helium being passed into contact with the ingot first in the series and thereafter successively to each of the remaining ingots in the series, thereafter cooling the ingots successively to substantially room temperature in said helium atmosphere while under said pressure, purifying the used helium to remove carbon dioxide, water vapor, hydrogen, oxygen and nitrogen therefrom, recycling the purified helium into contact with ingots under treatment in the series and removing said cooled ingots successively from said series.

GEORGE R. BURKHARDT.

#### REFERENCES CITED

The following references are of record in the file of this patent:

#### UNITED STATES PATENTS

| Number    | Name          | Date          |
|-----------|---------------|---------------|
| 314,004   | Edwards       | Mar. 17, 1885 |
| 1,842,200 | Ramage        | Jan. 19, 1932 |
| 2,057,518 | Fraser et al. | Oct. 13, 1936 |

#### FOREIGN PATENTS

| Number  | Country       | Date          |
|---------|---------------|---------------|
| 338,409 | Great Britain | Nov. 20, 1930 |